

Patented Feb. 2, 1932

1,843,200

# UNITED STATES PATENT OFFICE

JOHN WILLIAM BRANNON, OF ALSEA, OREGON

## METAL TEMPERING PROCESS

No Drawing.

Application filed August 19, 1930. Serial No. 476,454.

The invention aims to provide a new and improved process for hardening steel and iron of all grades with the aid of only a forge or other adequate heater, water, and an insulating or flux agent. This agent may consist of a mixture of powdered borax and powdered silica, powdered borax alone, or powdered silica alone. The process will be described and claimed using the expression "agent" and such expression is to be read in the light of the above definition. The steps are the same whether the agent be powdered silica alone, powdered borax alone, or a mixture of the two. The mixture preferably consists of two parts borax and one part silica.

The illustrations herein given will apply to carbon or tool steel, and to mild steel and iron, and other varieties of ferrous metals may be tempered in the same ways as herein explained.

The tempering of carbon or tool steel will be described in connection with a pre-formed tool which has been allowed to cool, but is obviously not restricted to tools. The tool is heated to a cherry red to a suitable distance from its point or edge, for example about three fourths of an inch or an inch back from said point or edge and is then dipped into or otherwise coated with the above mentioned agent. The agent clings to the tool and the coated tool is now further heated to a high cherry heat. It is then slowly dipped in cold water to a depth of about one half inch (or any depth required by the extent of temper required) and then quickly plunged entirely into and withdrawn from the water. This leaves sufficient heat in the tool to drive the temper down to the point or edge and the latter will show colors from straw to sky blue. These colors are generally known to indicate the degree of hardness to which the tool has been tempered, and when the proper color comes to the point or edge of the tool, I again plunge the latter in

the water. During the interval between the first and second plunges, the agent acts as an insulator and prevents too rapid cooling. The second plunge, when following the conventional way of tempering, causes trouble, for the tool will be harder back of the point or edge, but by using the insulating agent, the highest temper is insured at the point or edge. It has heretofore been proposed to use borax and the like to harden steel and iron but by my process, the borax, or other insulating agent performs the function of preventing hardening beyond the desired zone. When I dip the first time, I reserve enough heat to drive the temper down to the proper color and the insulating agent prevents the tool from cooling too quickly. Then I plunge the second time and by following these steps, I temper to the greatest extent where needed and overcome the undesirable element of tempering to a greater degree behind the point or edge with danger of breakage.

To harden mild steel or iron, the piece to be hardened, is heated to a cherry red or a little higher and dipped into the above described agent, the heat causing the agent to adhere to the metal. The coated metal is then reheated to the fusing point and cooled quickly in cold water. The agent acts now as a flux, causing the metal to run. This seals the grain or pores, solidifying the metal and producing when cooled, a hard product which is much tougher than carbon or tool steel.

Machine parts, tools and ferrous members of all descriptions, may be satisfactorily tempered according to the process herein disclosed and the tempering may be carried out without the aid of expensive ovens, furnaces or other apparatus.

I claim:

A process of tempering tool steel comprising the steps of heating the steel substantially to a cherry red, coating the heated steel with

the herein described agent (powdered borax, powdered silica, or both), reheating the coated steel to a high cherry heat, dipping the coated part slowly into water to the depth required by the extent of tempering desired, quickly plunging the steel into and removing it from the water, watching the color changes on the steel and when the sought color appears immersing the steel again in the water.

10 In testimony whereof I affix my signature.  
**JOHN WILLIAM BRANNON.**

**15****20****25****30****35****40****45****50****55****60****65**